

# United States Patent

Phillips, Jr.

[15] 3,692,888

[45] Sept. 19, 1972

[54] **CASTING HYDRIDES**

[72] Inventor: **Ernest C. Phillips, Jr.**, 2533 Albeworle Court, Richland, Wash. 99552

[22] Filed: **July 2, 1969**

[21] Appl. No.: **838,717**

[52] U.S. Cl. .... **264/5 R, 264/85, 264/332, 252/301.1 R, 23/204, 23/360, 117/5.3**

[51] Int. Cl. .... **G21c 21/00**

[58] **Field of Search**..... **264/85, 299, 332, 319, .5; 23/204, 360; 117/5.1, 5.3; 65/355; 252/301.1**

[56] **References Cited**

## UNITED STATES PATENTS

3,023,119 2/1962 Anderson et al. .... **117/5.1**

3,126,294 3/1964 Pichler ..... **117/5.3**  
3,224,860 12/1965 Stinnes ..... **65/355**

*Primary Examiner*—Carl D. Quarforth

*Assistant Examiner*—Stephen J. Lechert, Jr.

*Attorney*—Roland A. Anderson

[57]

## ABSTRACT

A method of casting lithium hydride, lithium deuteride or lithium tritide, or mixtures of these with zirconium hydride in a titanium or titanium-coated mold under a hydrogen atmosphere exceeding the dissociation pressure of titanium hydride, whereby, on cooling, the cast material can be readily removed from the mold without damage thereto.

**6 Claims, No Drawings**

## CASTING HYDRIDES

## BACKGROUND OF THE INVENTION

The invention described herein was made in the course of, or under, Contract No. AT(11-1)-GEN-8, with the United States Atomic Energy Commission.

This invention relates to a method of casting metal hydrides, particularly to casting of lithium hydride, lithium deuteride and lithium tritide, and more particularly to the casting of such materials in titanium or titanium-coated molds.

Prior to this invention, lithium hydride, deuteride, or tritide, which material is utilized, for example, as moderators for nuclear reactors and neutron shields, has been cast into iron, steel, or stainless steel molds to which the cast material adhered tenaciously. Removal of the cast material from such molds damages the surface of the material and often causes fractures in the material. Furthermore a thin layer of the cast material usually remains on the surface of the mold, thus requiring removal of this thin layer prior to subsequent reuse of the mold. Due to the surface damage of the cast material by the prior known molds, further finishing procedures have been required, thus increasing the costs.

While mold release coatings are known in the prior art, none of this prior known coatings have been found satisfactory for the casting of lithium hydride, deuteride or tritide.

## SUMMARY OF THE INVENTION

The process of this invention overcomes the problems of the prior art in the casting of lithium hydride, deuteride, or tritide by eliminating adherence between the mold and cast material, thereby producing a casting without damage to the surface thereof or fractures therein since the casting is not placed under stress by the mold during cooling and is readily removed from the mold. In addition, utilization of the present inventive casting method leaves the mold free of adhered casting material, thereby reducing the time and expense in the casting operation.

Therefore, it is an object of this invention to provide an improved method for casting lithium hydrides, deuteride and tritides.

Another object of the invention is to provide an improved casting method whereby the casted material is easily removed from the mold without damage to the cast material.

Other objects of the invention will become readily apparent from the following description of the improved casting process.

## DESCRIPTION OF THE INVENTION

As set forth above, lithium hydride, lithium deuteride, or lithium tritide, or mixtures of these with zirconium hydride has found numerous uses, especially in the nuclear field, as moderators for nuclear reactors and neutron shields. For such uses, castings of these materials in various desired shapes and with desired surface finishes are required. Such castings are readily produced in accordance with this invention by the utilization of titanium molds or molds of metals such as iron, steel or stainless steel which have been coated with titanium and casted as described hereinbelow.

During the casting process and during the cooling cycle, the mold and lithium hydride, for example, are kept under a hydrogen atmosphere, the pressure of which exceeds the dissociation pressure of titanium hydride. The time at temperature under the hydrogen atmosphere must be sufficient for the titanium to hydride and is, therefore, dependent upon the thickness of the titanium mold or titanium coating. Consequently, it is desirable to use the thinnest titanium practical. If sufficient time at temperature is not allowed, the titanium will acquire hydrogen, deuterium, or tritium from the cast material, leaving a small layer of metallic lithium between the mold and the casting, making it difficult to separate the casting from the mold.

During the casting process, usually at temperatures of 1,300° to 1,400° F, the titanium of the mold is partially hydrided. The cast lithium material has a greater coefficient of thermal expansion than the mold material (titanium) and does not adhere to the mold. During cooling, the cast lithium material shrinks more than the mold and separates from the mold. When cold, the mold and casting are easily separated. Since the cast lithium material does not adhere to the mold, the casting is not placed under stress by the mold during cooling, therefore, eliminating damage to the casting due to the mold. However, the surface finish of the casting is dependent upon the finish of the titanium surface of the mold.

By way of example only, the following operational sequence is set forth to provide a better understanding of the inventive casting method.

1. Molten lithium hydride, deuteride or tritide is poured into a titanium or titanium-lined mold.
2. The mold is placed in a furnace having a temperature maintained at approximately 1,300° to 1,400° F and in a hydrogen atmosphere exceeding the dissociation pressure of titanium hydride, the cast material having a greater coefficient of thermal expansion than the mold and thus does not adhere to the mold.
3. The furnace temperature and hydrogen pressure are maintained for a period of time sufficiently long to convert the titanium to titanium hydride, the time being dependent on the thickness of the titanium utilized.
4. The mold is cooled while maintaining the hydrogen atmosphere pressure to prevent dissociation of the titanium hydride wherein the casting shrinks more than the mold and does not place any stress on the casting during cooling.
5. After cooling, removal of the casting from the mold is facilitated by the shrinking of the casting which separates same from the mold. Since there is no adherence between the mold and the casting, the surface of the casting is not damaged and the casting is not placed under any stress during the cooling, thereby eliminating damage to both the casting and the mold.

The following examples illustrate tests carried out utilizing the hereinbefore described inventive method:

## EXAMPLE I

A piece of titanium tubing was used as a mold. During the casting an atmosphere of hydrogen at a pressure

of about 860 mm Hg absolute was maintained. Lithium hydride was cast and, after cooling, was readily removed from the mold. In tests performed as directly about but with insufficient hydrogen present there was severe sticking of the casting to the mold, and the hydride cracked on cooling due to the adherence of the periphery thereof to the mold and to the resulting tensile stresses.

#### EXAMPLE II

A mild steel mold was coated with a very thin layer of titanium by evaporation in vacuum. Again, lithium hydride was successfully cast under an atmosphere of hydrogen (same pressure) and easily removed from the mold. In similar tests with a mild steel mold, it was found that when either the titanium coating or the hydrogen atmosphere was omitted, sticking occurred.

#### EXAMPLE III

A mold of stainless steel was coated and used in Example II above with the same results. Tests with the stainless steel mold showed that sticking occurred as with the mild steel mold when either the titanium coating or the hydrogen atmosphere was omitted.

Although only lithium hydride, deuteride or tritide have been specifically considered in the description of inventive method, it is believed that calcium hydride could be cast by this process. While high melting hydrides, such as zirconium hydride would probably not cast satisfactorily; a mixture of lithium hydride, deuteride or tritide with zirconium hydride may be cast in accordance with the invention.

While the titanium or titanium-coated mold may be pre-treated with hydrogen to form a hydrided surface before carrying out the casting operation, this is not necessary since the hydrogen diffuses so rapidly through the lithium hydride, for example, and apparently even along very thin coatings of titanium, that it performs its intended function even when the mold is 40 filled with lithium hydride.

It has been shown that the present invention provides

an improved method for casting materials and particularly for casting lithium hydride, deuteride or tritide.

Although specific parameters for the inventive casting method have been described, modifications will 5 become apparent to those skilled in the art, and it is intended to cover in the appended claims all such modifications as come within the spirit and scope of the invention.

I claim:

- 10 1. A method of casting materials comprising the steps of: containing a casting material selected from the group consisting of lithium hydride, lithium deuteride, and lithium tritide in a mold at least lined with a layer of titanium, heating the thus contained casting material 15 to a temperature so that the titanium of the mold is at least partially hydrided and in a hydrogen atmosphere having a pressure greater than the dissociation pressure for a time period sufficiently long to convert the titanium to titanium hydride, cooling the thus cast material 20 while maintaining the hydrogen pressure to prevent dissociation of the titanium hydride, and removing the casting from the mold.
2. The method defined in claim 1, additionally including the step of coating the layer of titanium on a mold formed of metal selected from the group consisting of iron, mild steel and stainless steel.
3. The method defined in claim 1, wherein the heating temperature is maintained in the range of about 1,300° to 1,400° F.
- 30 4. The method defined in claim 1, wherein the hydrogen atmosphere is maintained at a pressure of about 860 mm Hg absolute.
5. The method defined in claim 1, wherein the material to be cast from the selected group is mixed 35 with zirconium hydride prior to the step of containing the casting material in the titanium lined mold.
6. The method defined in claim 1, additionally including the step of pre-treating the titanium lined mold with hydrogen forming a hydrided surface thereon prior to containing and heating the casting material therein.

\* \* \* \* \*